# EUROPEAN PATENT SPECIFICATION

(11) **EP 0 819 790 B1**
(45) Date of publication and mention of the grant of the patent: **12.12.2001**
(21) Application number: 97202155.4
(22) Date of filing: 09.07.1997
(51) Int. Cl.: D06N 7/00, D06N 3/14, D06N 3/00, D06N 3/04, B32B 27/12

(54) **Cloth structure**
Gewebestruktur
Structure tissée

(30) Priority: 09.07.1996 NL 1003545
(43) Date of publication of application: 21.01.1998
(73) Proprietor: Prof B.V., 7731 TK Ommen (NL)
(72) Inventor: De Bie, Erik, 7451 JL Holten (NL)
(74) Representative: Schumann, Bernard Herman Johan

(56) References cited:
- EP-A- 0 073 948
- EP-A- 0 151 963
- EP-A- 0 364 370
- WO-A-88/01570
- US-A- 4 547 423
- US-A- 4 816 328
- US-A- 5 017 424
- DATABASE WPI Section Ch, Week 9513 Derwent Publications Ltd., London, GB; Class A25, AN 95-094347 XP002026987 & JP 07 018 584 A (DAIICHI LACE KK) , 20 January 1995

## Description

The invention relates to a cloth structure, comprising:
a base cloth serving as a middle layer, which base cloth consists substantially of polyester multifilaments and/or microfilaments and/or staple fibres, and contains electrically conducting and thus antistatic fibres such that the base cloth is antistatic, which fibres consist for instance of carbon and are preferably ordered in a check structure;
a microporous and/or hydrophilic, fire-retardant and flame extinguishing first cover layer arranged on the inside of the base cloth, which first cover layer consists substantially of a microporous and/or hydrophilic polyurethane and/or polytetrafluoroethylene;
a second cover layer arranged on the outside of the base cloth.

Such a structure is known from US-A-4 547 423.

EP-A-0 073 948 describes a cloth structure comprising a base cloth serving as middle layer and a first cover layer arranged on the inside and a second cover layer arranged on the outside of the base cloth. The base cloth can be made out of polyesther fibres or carbon fibres. In order to provide the cloth structure with several properties the first and second cover layer can contain hydrophilic polymers, such as polyurethane, which is blended with several other components which provide the desired properties. In order to give the cloth structure a certain color, colorants are added to the polymer.

The invention has for its object to provide a cloth structure which is watertight, windtight, flame-retardant, resistant to chemicals, antistatic and permeable for water vapour.

In respect of the above the invention generally provides a cloth structure, which is characterized by a second cover layer comprising a predominant portion of fluorocarbon resin who's fire resistance compiles with the index according to EN 532/533, and the base cloth being colored with fluorescent colorants which provide increased visibility.

An embodiment is recommended in which the base cloth consists predominantly of polyester fibres and/or polyester filaments.

In respect of said properties it is of the greatest importance, particularly for safety clothing for instance for the petrochemical industry, that there is no danger of static charging of the cloth structure which could result in spark formation. In respect thereof a preferred embodiment has the special feature that the base cloth contains electrically conducting and thus antistatic fibres such that the base cloth is antistatic, which fibres consist for instance of carbon and are preferably ordered in a check structure.

An example of such a structure is that wherein in the base cloth a woven material is incorporated which is known as "Kanebo antistatic check".

As composition a base cloth can for instance be envisaged which in total constitutes 48% of the cloth and consists of polyester micro-fibre, together with 2% Kanebo antistatic check, while said cover layers consist respectively of a number of flame-extinguishing products totalling 10% and 40% polyurethane. The specific weight can be in the order of (195 ± 50) g/m².

A water column of more than two 2 m. does not yet produce any seepage of water. This relates to the cloth structure both in new condition and after washing ten times at 60°C. The water vapour permeability is for instance greater than 600 g/m²/24h. The fire class corresponds with the French norm M1 and the European norm EN 533.

A specific embodiment has the special feature that the base cloth contains a woven material.

Alternatively an embodiment can be envisaged in which the base cloth comprises a non-woven.

A specific embodiment has the special feature that the first cover layer consists at least predominantly of polyurethane.

A variant can also be envisaged in which the two cover layers coincide. In particular, the two cover layers can together predominantly consist of polyurethane.

Yet another embodiment has the special feature that a flame-retardant agent is added to the polyurethane, for instance a halogen-free or brominated hydrocarbon and/or a nitrogen and/or phosphorus-containing compound such that the relevant cover layer is flame-retardant.

The base cloth as specified in claim 6 in particular can be made fireproof on the basis of a halogen-free, fire-retardant aqueous solution of inorganic or organic nitrogen and/or phosphorus compounds posing no hazards for human beings and environment. Below are given some examples of compounds for elucidation of the terminology used.

The compound (1) is an organic nitrogen compound, that is, aniline.

The compound (2) is likewise an organic nitrogen compound, that is, nitrobenzene.

The compound (3) is likewise an organic nitrogen compound, that is, n-propylamine.

CH₃-CH₂-CH₂-NH₂ (3)

The compound (4) is a cobalt complex, an inorganic nitrogen compound.

The compound (5) is triphenylphosphine, an organic phosphorus compound.

The compound (6) is aluminium phosphate, an inorganic phosphorus compound.

AlPO₄ (6)

The compound (7), finally, is a brominated hydrocarbon, that is, 2-bromobutane.

It will be apparent that the cloth structure according to the invention can be embodied and varied in diverse ways. In addition, the structure can possess other than the stated properties. It can for instance be strongly wear-resistant, have great stretch resistance, be resistant to high and low temperatures, be provided with particular colours and so on.

The cloth structure according to the invention lends itself extremely well for application in CE approved safety clothing designed for single or combined, diverse and unrelated or interrelated hazards.

In a preferred embodiment the invention has for its object to provide a cloth structure which mutually combines a plurality of technical properties. The object of the invention in this aspect is to provide a cloth structure which combines at least a number of the following properties: watertight, permeable for water vapour, windtight, flame-retardant, resistant to chemicals, antistatic and increased visibility. This combination of properties is not known from the literature since, in contrast to the prior art, conflicting functions must be combined in one cloth structure.

According to a first aspect of this part according to the invention the cloth structure comprises:
the base cloth serving as middle layer;
a microporous and/or hydrophilic first cover layer arranged thereon on the inside; and
a second cover layer arranged thereon substantially on the outside and comprising a predominant proportion of fluorocarbon resin.

This cloth structure preferably displays the special feature that the base cloth consists substantially of polyester multifilament and/or microfilament and/or staple-fibres.

This cloth structure preferably has the special feature that the base cloth consists substantially of polyester fibres.

This latter variant can advantageously be applied for the use of fluorescent colours which for instance may greatly improve the safety of a user. In this respect the invention provides in this aspect a cloth structure in which the base cloth is coloured with colorants which provide increased visibility, in particular fluorescent colorants.

A polyester woven material is however not electrically conducting, whereby, when used as protective clothing in an explosion-hazardous environment, spark-over is possible as a result of static electrical charging of the clothing, which could cause an explosion and is therefore not acceptable. This can be obviated by applying conductive fibres, particularly in a check structure in the woven material, whereby the build-up of static electricity is effectively prevented. In practice this step is found to be effective, even if cover layers are arranged on both sides of the base cloth.

A specific embodiment has the special feature that the first cover layer consists substantially of a microporous and/or hydrophilic polyurethane and/or polytetrafluoroethylene.

A specific embodiment hereof displays the feature that the first cover layer is applied by a coating process or a laminating process on the basis of a film. The first cover layer preferably has a colour which depends on the colour of the base cloth. This is of particular importance in respect of the effect on a possible fluorescent colour of the base cloth. In the case the base cloth has such a fluorescent colour, the cover layer is preferably clear white. In other cases the cover layer can have the colour of the base cloth.

As already discussed above, the cover layer can take a flame-retardant form, for instance comprise flame-retardant agents. These can for instance be based on nitrogen and/or phosphorus compounds or organobromine compounds. The concentrations of these flame-retardant agents in the cover layer must be sufficient to impart flame-retardant properties to the total cloth structure, also in combination with an optionally untreated base cloth. On the other hand, it must be taken into account that the concentrations of the flame-retardant agents in the cover layer may not be so high that this results in an adverse effect on the achieved water vapour permeability, the strength and the wear-resistance of the cover layer.

The outer cover layer also functions as barrier against water or other liquids coming from outside, to which the protective clothing based on the cloth structure according to the invention may be exposed during operational conditions. Due to the hydrophilic and/or microporous character the cover layer is permeable for water vapour. By its nature the base cloth is likewise so, so that the total cloth structure is thereby permeable for water vapour.

In respect of the water vapour permeability it is noted that this is inversely proportional to the water vapour resistance, which will be further mentioned hereinbelow.

The cover layer can be deemed completely windtight.

Brief attention will now be given to the second cover layer. This second cover layer is predominantly arranged on the outside, for instance by means of a spray, dip or brush technique. It comprises a predominant proportion of fluorocarbon resin and can even substantially consist thereof.

The "inside" and "outside" are defined in terms of the inside and outside of the protective clothing manufactured on the basis of the cloth structure according to the invention.

The second cover layer ensures repulsion of for instance splashes of liquid chemicals of for instance the most frequently occurring types or specific types for which the cloth structure is designed. In combination with the first cover layer, these splashes are prevented from passing through the cloth structure. The second cover layer is very thin. Hereby is prevented that this cover layer will have an adverse effect on the water vapour permeability.

With the combination of the above described steps the following properties are obtained:

| **Property** | **Value** |
|---|---|
| Watertightness | ≥13 kPa ISO 811 |
| Water vapour resistance | ≈ 150 m² Pa/W |
| Airtightness | ≈ 20 1 m²/s |
| Fire resistance | index according to EN 532/533 |
| Antistatic properties | complies with EN 1149-1 |
| Increased visibility | complies with EN 471 |
| Chemical resistance | penetration index = 0.0% |
| (kerosine) | Repulsion index ≥ 95% according to EN 368 |

It is again noted that the literature provides no single indication relating to the combination of the above stated properties. JP-A-0 516 684 for instance mentions a cloth structure having a PVC-like character and intended as artificial leather. This cloth structure is essentially non-breathing.

A fire-retardant cloth structure is known per se from for instance DE-A-41 32 427.

The annexed figure shows in cross section a part of the cloth structure 1 according to the invention. The outside of the cloth is designated with the reference numeral 2, while the reference numeral 3 refers to the inside.

The base cloth 4 is some tenths of a millimetre thick. It consists of polyester multi-, microfilament or staple fibres which are treated with a colorant to provide the cloth structure with the desired colour. Arranged on the outside 2 is a second cover layer 5 which is a few micrometers thick and consists of a fluorocarbon resin.

Arranged on the inside 3 is a microporous and/or hydrophilic, flame-retardant first cover layer 6 with a thickness of some tenths of a millimetre. This cover layer 6 for instance consists wholly or partially of polyurethane, which is transparent by nature, or polytetrafluoroethylene, which is white by nature. The base cloth comprises a woven material of yarns or threads, respectively 7 in the warp direction and 8 in the weft direction. The threads are replaced locally in both directions by electrically conducting yarns or threads 9, consisting for instance of carbon fibres.

It is noted that the drawing is not necessarily drawn to scale.

Further attention is drawn to the fact that the drawing is highly schematic and that the first cover layer 6 can for instance follow the contours of base cloth 4 more closely.

It is further pointed out that the form of the second cover layer 5 is shown very schematically. It is the intention of the drawing to make clear that this layer, which can for instance be applied by spraying, will adapt naturally to the form of base cloth 4.

Said antistatic threads, filaments, fibres or yarns may also consist of materials other than carbon, for instance conductive metals or composite materials. They are co-woven with a suitable weaving technique and thereby form part of the woven material.

## Claims

1. Cloth structure (1), comprising:
a base cloth (4) serving as a middle layer, which base cloth (4) consists substantially of polyester multifilaments and/or microfilaments and/or staple fibres, and contains electrically conducting and thus antistatic fibres (9) such that the base cloth is antistatic, which fibres (9) consist for instance of carbon and are preferably ordered in a check structure;
a microporous and/or hydrophilic, fire-retardant and flame extinguishing first cover layer (6) arranged on the inside of the base cloth (4), which first cover layer (6) consists substantially of a microporous and/or hydrophilic polyurethane and/or polytetrafluoroethylene;
a second cover layer (5) arranged on the outside of the base cloth (4),
**characterized by**
the second cover layer (5) comprising a predominant portion of fluorocarbon resin whose fire resistance compiles with the index according to EN 532/533, and the base cloth (4) being colored with fluorescent colorants which provide increased visibility.

2. Cloth structure (1) as claimed in claim 1, wherein the base cloth (4) contains a woven material.

3. Cloth structure (1) as claimed in claim 1, wherein the base cloth (4) comprises a non-woven.

4. Cloth structure (1) as claimed in claim 1, wherein the base cloth (4) is impregnated with a flame-retardant agent, for instance a halogen-free or brominated hydrocarbon and/or a nitrogen and/or phosphorus-containing compound such that the base cloth is flame-retardant.

5. Cloth structure (1) as claimed in claim 1, wherein a flame-retardant agent is added to the polyurethane, for instance a halogen-free or brominated hydrocarbon and/or a nitrogen and/or phosphorus-containing compound such that the relevant cover layer (5, 6) is flame-retardant.

6. Cloth structure (1) as claimed in claim 1, wherein the first cover layer (6) is applied by a coating process or a laminating process on the basis of a film.

## Patentansprüche

1. Gewebestruktur (1), die umfasst:
eine als eine mittlere Schicht dienende Grund-Gewebestruktur (4), wobei die Grund-Gewebestruktur (4) im wesentlichen aus Polyester-Multifilamenten und/oder -Microfilamenten und/oder -Spinnfasern besteht, und elektrisch leitende und somit antistatische Fasern (9) enthält, so dass das Grundgewebe antistatisch ist, wobei die Fasern (9) beispielsweise aus Kohlenstoff bestehen, und vorzugsweise zu einer Check-Struktur geordnet sind;
eine mikroporöse und/oder hydrophile, feuerhemmende und flammenauslöschende erste Bedeckungsschicht (6), die auf der Innenseite der Grund-Gewebestruktur (4) angebracht ist, wobei die erste Bedeckungsschicht (6) im wesentlichen aus einem mikroporösen und/oder hydrophilen Polyurethan und/oder Polytetrafluorethylen besteht;
eine zweite Bedeckungsschicht (5), die auf der Außenseite der Grund-Gewebestruktur (4) angebracht ist,
**dadurch gekennzeichnet, dass**
die zweite Bedeckungsschicht (5) einen vorherrschenden Anteil eines Fluorkohlenwasserstoffharzes umfasst, dessen Feuerbeständigkeit dem Index gemäß EN 532/533 entspricht, und die Grundgewebestruktur (4) mit fluoreszierenden Farbstoffen, die eine erhöhte Sichtbarkeit bereitstellen, gefärbt ist.

2. Gewebestruktur (1) wie in Anspruch 1 beansprucht, wobei die Grund-Gewebestruktur (4) ein gewebtes Material enthält.

3. Gewebestruktur (1) wie in Anspruch 1 beansprucht, wobei die Grundgewebestruktur (4) ein Vlies umfasst.

4. Gewebestruktur (1) wie in Anspruch 1 beansprucht, wobei die Grund-Gewebestruktur (4) mit einem flammenhemmenden Mittel, zum Beispiel einem halogenfreien oder bromierten Kohlenwasserstoff und/oder einer Stickstoff und/oder Phosphor enthaltende Verbindung so imprägniert ist, dass das Grundgewebe flammenhemmend ist.

5. Gewebestruktur (1) wie in Anspruch 1 beansprucht, wobei ein flammenhemmendes Mittel, beispielsweise ein halogenfreier oder bromierter Kohlenwasserstoff und/oder eine Stickstoff und/oder Phosphor enthaltende Verbindung zu dem Polyurethan so hinzugefügt wird, dass die relevante Bedeckungsschicht (5, 6) feuerhemmend ist.

6. Gewebestruktur (1), wie in Anspruch 1 beansprucht, wobei die erste Bedeckungsschicht (6) durch ein Beschichtungsverfahren oder ein Laminierungsverfahren auf der Basis einer dünnen Schicht aufgetragen wird.

## Revendications

1. Structure tissée (1), comprenant :
un tissu de base (4) servant de couche intermédiaire, tissu de base (4) qui est constitué essentiellement de multifilaments et/ou de microfilaments et/ou de fibres discontinues de polyester, et contient des fibres (9) conduisant l'électricité et, par conséquent, antistatiques, de telle sorte que le tissu de base soit antistatique, fibres (9) qui sont constituées, par exemple, de carbone et sont disposées, de préférence, suivant une structure quadrillée ;
une première couche de couverture (6) microporeuse et/ou hydrophile, retardatrice de feu et extinctrice de flammes, disposée à l'intérieur du tissu de base (4), première couche de couverture (6) qui est constituée essentiellement de polyuréthane et/ou de polytétrafluoroéthylène microporeux et/ou hydrophile ;
une deuxième couche de couverture (5) disposée à l'extérieur du tissu de base (4)
**caractérisée par le fait que**
la deuxième couche de couverture (5) comprend une partie prédominante de résine de fluorocarbone dont la résistance au feu satisfait aux normes EN 532/533, et que le tissu de base (4) est coloré avec des colorants fluorescents pour le rendre plus visible.

2. Structure tissée (1) selon la revendication 1, dans laquelle le tissu de base (4) contient une matière tissée.

3. Structure tissée (1) selon la revendication 1, dans laquelle le tissu de base (4) comprend une matière non-tissée.

4. Structure tissée (1) selon la revendication 1, dans laquelle le tissu de base (4) est imprégné d'un agent retardateur de flammes, par exemple un hydrocarbure dépourvu d'halogène ou bromé et/ou un composé contenant du phosphore et/ou de l'azote, de telle sorte que le tissu de base soit retardateur de flammes.

5. Structure tissée (1) selon la revendication 1, dans laquelle un agent retardateur de flammes est ajouté au polyuréthane, par exemple un hydrocarbure dépourvu d'halogène ou bromé et/ou un composé contenant du phosphore et/ou de l'azote, de telle sorte que la couche de couverture (5, 6) soit retardatrice de flammes.

6. Structure tissée (1) selon la revendication 1, dans laquelle la première couche de couverture (6) est appliquée suivant un procédé d'enduction ou un procédé de laminage sur la base d'un film.
